

Dec. 27, 1949

D. C. FONDA

2,492,214

METHOD OF MARKING TUNGSTEN CARBIDE

Filed Oct. 25, 1945



## UNITED STATES PATENT OFFICE

2,492,214

## METHOD OF MARKING TUNGSTEN CARBIDE

Douglass C. Fonda, Stamford, Conn.

Application October 25, 1945, Serial No. 624,432

3 Claims. (Cl. 204—143)

1

This invention relates to the marking of legends, such as size designations, on articles made of tungsten carbide.

Conventional methods of marking steel parts cannot be used effectively on tungsten carbide which resists the action of acids that are used for etching. Tungsten carbide can be marked with diamonds, but the process is costly, so costly in fact that it has been the practice to sell tungsten carbide parts without size designations.

It is an object of this invention to provide an improved method for marking tungsten carbide parts. The invention is convenient to use, marks the parts quickly and is economical. Although it will be described in connection with the marking of gage blocks, the invention is suitable for marking tungsten carbide parts generally.

The process of this invention utilizes an electric current passed through a liquid electrolyte, preferably an acid, that contacts with the surface to be etched only along the lines of the marks to be made.

Other objects, features and advantages of the invention will appear or be pointed out as the description proceeds.

In the drawings, forming a part hereof, in which like reference characters indicate corresponding parts in all the views,

Figure 1 is a diagrammatic sectional view showing a tungsten carbide element coated with a resist, and illustrating the way in which markings are made through the resist with a scribe.

Figure 2 is a large-scale side view, mostly in section, showing the process of marking a tungsten carbide gage block in accordance with this invention.

Figure 3 is a front elevation on a reduced scale, showing the gage block of Figure 2 after it has been marked.

In carrying out the process of this invention for marking tungsten carbide gage blocks, a coating of resist 11 is first applied to the surface that is to be marked. Although no electrolyte comes in contact with the sides of the block when the process is carried out in the intended manner, the coating of resist is preferably applied to the sides of the block also as a protection since some electrolyte may accidentally run down the sides. The resist is a non-conductor of electricity and usually a finely ground powder carried by a vehicle, for example carbon tetrachloride. Commercial products are available on the market, one such resist is "Holsapple's Ground."

In order to etch a fine line, such as is used for gage block marking, it is necessary that the resist be made of finely ground material so that a thin line can be cut through the resist by means of a scribe or stylus 13. The scribe 13 is preferably moved by a pantograph which operates against letter or numeral guides for ob-

15 taining perfect letters or figures. The line cut in the resist by the scribe is designated in Figure 1 by the reference character 14.

After the necessary inscriptions have been cut through the resist coating 11, a drop of liquid 17 is placed on the resist over the lines made by the scribe. The block 10, which is to be marked at an upper end with a size designation, and below its mid region with the manufacturer's name and a serial number, is shown in Figure 2 with two globules of liquid 17 placed in position to cover the areas of the markings.

It is unnecessary to spread the liquid 17 over areas of the block that are not to be marked, but no harm is done in having such areas covered by the liquid 17 since the resist prevents the liquid from coming in contact with the metal of areas not exposed by the scribe. When etching gage blocks one drop of liquid is used for each line of marking, or a large drop for two lines located close together, and it is advantageous to apply the liquid as drops or globules so that the liquid does not flow beyond the edges of the resist and down over the side surfaces of the block.

20 The liquid 17, which serves as an electrolyte during its etching process is preferably an acid, but other liquids can be used, even water.

In order to etch the block a pointed electrode 20 is brought into contact with one of the drops of electrolyte 17 and a high intensity current at low voltage is passed from the electrode 20 through the electrolyte 17 to the block 10. The uncoated bottom surface of the block 10 rests on a metal support 21 that is connected in the circuit with the electrode 20. The power is ordinarily supplied from a transformer 22 in which the voltage can be stepped down from that of a primary supply source 24.

25 The electrode 20 shown in Figure 2 has a pointed end, but it is not essential that the end of the electrode be pointed. It is a feature of the invention, however, that the electrode is brought into contact with the drop or globule 17 of the electrolyte but not with the coating of resist 11. The disadvantage of touching the electrode to the coating 11 is that the coating is likely to be broken by the mechanical contact, and the distribution of current through the regions cut in the resist is more uniform if the electrode 17 is merely brought into contact with the upper portion of the globule 17.

30 It is not essential that the electrode touch the globule 17 in the middle, and in the operation illustrated in Figure 2 the electrode 20 is shown in contact with one side of the globule 17. With a dilute acid globule and a current of 25 amperes, it is necessary to maintain the electrode 20 in contact with the electrolyte 17 for only one or two seconds in order to mark the gage block.

Using water as the electrolyte increases the time to a period of from six to ten seconds. The secondary voltage of the transformer 22 for these illustrations is 12 volts. These values are given as merely illustrative. Longer periods of current flow result in deeper etching of the tungsten carbide surface. For marking gage blocks, thin lines without deep etching tend to keep the block from warping, they are considered more attractive in appearance, and they have the practical advantage that less subsequent lapping of the block is required to remove any upset of the metal caused by the etching operation.

Experience has shown that this process produces legends around which there is no noticeable burr or upset unless the surface is subjected to the exacting scrutiny of the optical instruments used in testing the flatness of gage blocks.

With such instruments a slight upset is found along the edges of the etched legends, and in gage block manufacture the etching is therefore done after the rough lapping and before the final finish lapping of the surfaces of the blocks.

The electrode 20 is applied to the globules 17 by hand, and it is provided with a coating of insulation 26 that provides a convenient handle by which the electrode can be gripped by the operator using it. The electrode 20 is preferably made of brass and the handle 26 of rubber, wood or other insulating material which is light and easily held.

When the current has flowed through the globule 17 long enough to etch the tungsten carbide, the electrode is removed and the globule 17 is blotted off the surface. The block is then washed in naphtha or any other suitable liquid for removing the coating of resist 11. Figure 3 shows the block after the resist has been removed and shows the regions etched in the block by the passage of the heavy electric current.

The preferred embodiment of the invention has been illustrated and described, but changes and modifications can be made and the current applied in ways other than those illustrated without departing from the invention as defined in the claims.

I claim as my invention:

1. The method of marking tungsten carbide gage blocks, which method comprises coating the gage block with a resist after the block has been rough lapped and before the final lapping of the block to size, marking a size designation or other symbol through the resist over a relatively small area of the block by means of a sharp pointed scribe, placing liquid electrolyte over the marks cut through the resist by said scribe, the liquid electrolyte being limited to a globule that has a generally convex top surface maintained at a substantial distance above the surface of the resist by the surface tension of the liquid electrolyte, bringing the point of a metal electrode into contact with the electrolyte over an area substantially less than the area of contact of the globule with the block and without touching the resist or the gage block, passing an electric current from the electrode through the electrolyte to the surface of the gage block exposed through the markings cut in the resist, continuing the flow of current until the block is marked to the desired depth, and thereafter lapping the block to final gaging dimensions and flatness.

2. The method of marking size designations and other legends on a relatively small area of the gaging surfaces of tungsten carbide gage blocks, which method comprises coating a gaging surface of the block with a resist after the block has been rough lapped and before the final lapping of the gaging surfaces, cutting fine outlines of the numerals or other legends to be etched in the block by means of a sharp pointed scribe that pierces the resist and bears against the metal of the face to be etched, placing a drop of electrolyte over each line of legends cut by the scribe to form globules of liquid on the resist, each drop of liquid electrolyte being limited to a globule that has a generally convex top surface maintained at a substantial distance above the surface of the resist by the surface tension of the liquid electrolyte, which globules terminate short of the edges of the block, bringing a point of a metal electrode into contact with each drop of liquid successively over an area substantially less than the area of contact of the globule with the block, holding the electrode out of contact with the resist and the metal of the block, passing an electric current of approximately 25 amperes from the electrode through the electrolyte to the metal exposed through the lines cut through the resist for a period of approximately two seconds, removing the electrode, blotting the globules of liquid from the block, washing the resist from the block and thereafter lapping the block to remove the metal upset by the etching process.

3. The method of marking tungsten carbide parts, which method comprises coating the part with resist, marking a size designation or other symbol through the resist, over a relatively small area of the part, by means of a sharp-pointed scribe, placing a liquid electrolyte over the marks cut through the resist by said scribe, the liquid electrolyte being limited to a globule that has a generally convex top surface maintained at a substantial distance above the surface of the resist by the surface tension of the liquid electrolyte, bringing the point of a metal electrode into contact with the electrolyte over an area substantially less than the area of contact of the globule with the part and without touching the resist or the tungsten carbide part, passing an electric current from the electrode through the electrolyte to the surface of the part exposed through the markings cut in the resist, and continuing the flow of current until the block is marked to the desired depth.

DOUGLASS C. FONDA.

#### REFERENCES CITED

The following references are of record in the file of this patent:

#### UNITED STATES PATENTS

| Number    | Name       | Date           |
|-----------|------------|----------------|
| 534,895   | Legate     | Feb. 26, 1895  |
| 1,376,365 | Wertheimer | Apr. 26, 1921  |
| 1,844,928 | Slepian    | Feb. 9, 1932   |
| 2,385,198 | Engle      | Sept. 18, 1945 |

#### OTHER REFERENCES

"Zeitschrift fur Metallkunde," vol. 16 (April 1924), pages 132, 133.